

July 24, 1928.

1,677,973

F. F. MARQUARD

## METHOD OF QUENCHING COKE

Filed Aug. 8, 1925

2 Sheets-Sheet 1

*Fig. 1.*



*Witnesses:*

Edwin Trubé

*Inventor:*  
FRANK F. MARQUARD,

by: *Anthony J. Esma*  
*Anthony J. Esma*  
his Attorney

July 24, 1928.

1,677,973

F. F. MARQUARD

METHOD OF QUENCHING COKE

Filed Aug. 8, 1925

2 Sheets-Sheet 2

*Fig. 2.*



Witnesses:

*Edwin Truelb*

Inventor:

By: *FRANK F. MARQUARD,*  
*D. Anthony Lewis*  
*his Attorney.*

## UNITED STATES PATENT OFFICE.

FRANK F. MARQUARD, OF CLAIRTON, PENNSYLVANIA.

## METHOD OF QUENCHING COKE.

Application filed August 8, 1925. Serial No. 49,038.

This invention relates to the manufacture of coke and more particularly to a novel method of quenching hot coke after it is discharged from the coke ovens, and has for 5 one of its objects the provision of a novel method of quenching whereby the coke is reduced to a comparatively uniform temperature and is free from hot spots.

Another object is to provide an improved 10 method of quenching coke whereby the final moisture content of the coke is very much reduced resulting in an improved quality of coke.

Another object is to provide an improved 15 method of quenching coke whereby less water is required for the quenching operation due to the more efficient application of the water.

A further object is to provide an improved 20 method of quenching coke whereby effectiveness of the quenching water recirculated in a closed system is increased due to remaining at a lower temperature. The fact that less excess water is used, less water is drained 25 back into the system.

Heretofore the hot coke has been discharged from the coke ovens into a car, commonly known as a hot car or quenching car. The car then is conveyed to a quenching station consisting of a suitable tower of 30 sufficient size to receive the car, and a system of water sprays. When the car has been placed in the quenching tower, or station, the sprays are operated so as to continuously 35 spray the hot coke in the car with water for 30 to 75 seconds at the rate of from 150 to 200 gallons of water per second. This continuous spraying resulted in a flooded hot car, and the excess of water in the car interfered with the free passage of air and 40 water vapors and greatly reduced the efficiency of the quenching operations. Many effects detrimental to the quality of the coke and life of the equipment resulted from the flooding of the hot car. Owing to variations 45 in operations, the coke was not uniformly spread throughout the length of the hot car and due to irregularities in oven temperatures, some coke was much hotter than other 50 coke of the same charge. Since there was no practical way of varying the water spray to vary the thickness and temperature of coke in the car, frequently red hot coke would remain in parts of the car while the 55 coke in other parts of the car would be over-quenched. Over-quenching of the coke re-

sults in a high moisture content which is very undesirable for metallurgical purposes. Furthermore, over-quenched coke screens 60 poorly, due to the coke dust and small particles clinging to the moist pieces of coke, resulting in what is known as dirty coke.

The under-quenched or hot coke requires the additional labor for spot quenching by 65 hand hose on the coke wharf, and even then portions of the hot or under-quenched coke is liable to be discharged onto the conveyers leading to the storage bins or cars, resulting in damage to such conveyers and, at times, in the igniting of the coke in the bin or car. 70

Attempts heretofore have been made to prevent the two extremes of over and under-quenching the coke, by varying the number and size of spray holes and varying the time 75 of spraying, but all of such attempts have utilized a continuous spraying or flooding of the coke.

The improved method of this application follows the usual method up to the time the quenching or hot car enters the quenching 80 tower, and utilizes the same or substantially the same apparatus used in carrying out the old method. After the quenching or hot car is positioned in the quenching tower the coke is sprayed with water at the rate of from 85 150 to 200 gallons per second for a very short period of approximately five seconds, and then allowed to drain for a more extended period of approximately thirty seconds, and then again sprayed with water at the rate of 90 from 150 to 200 gallons per second for a period of approximately five seconds, and again allowed to drain for a period of approximately thirty seconds. This alternate spraying and draining may be continued until the coke 95 is entirely quenched, although generally two quenching and draining periods are sufficient to completely quench the usual charge of coke in a quenching car.

In this manner, after each short interval 100 of quenching, the coke is allowed to drain and all water retained by the coke is evaporated, allowing the maximum cooling effect, due to the free passage of the water vapor and air between the pieces of coke and the free interchange of heat between the various parts of the charge of coke, resulting in the charge of coke being quenched to a comparatively uniform temperature throughout, and having a low average moisture content. 105

In the drawings:  
Figure 1 is a sectional end elevation of

a quenching tower adapted to carry out my invention.

Figure 2 is a sectional side elevation thereof.

5 Referring more particularly to the drawings the numeral 2 designates the tower as a whole which is generally of rectangular shape and is provided with an opening 3 in each end wall to permit the entrance and 10 exit of the quenching car 4. The tower is of sufficient size to receive and enclose the quenching car.

The quenching car 4 may be of any ordinary standard construction and is generally 15 provided with an inclined bottom wall 5 to permit the gravity discharge of the quenched coke, and perforated side walls (not shown) to permit the discharge of the excess sprayed water.

20 A suitable sump 6 is provided along one side wall of the tower and a drain outlet opening 7 along the bottom of the tower permits the excess water drained from the car 4 to escape through the opening 7 into the 25 sump.

A suitable supply pipe 8 is arranged to supply water to the sump 6 and a pipe 9 leads from the sump to a pump 10, which pump operates to draw water from the sump 30 and force it up through a conduit 11 to a tank 12 from which it is discharged through a discharge conduit 13 to the spray pipes 14 having suitable openings (not shown) through which the water is sprayed onto 35 the hot coke in the car 4. A valve 15 is located intermediate the ends of the conduit 13 to control the flow of water to the spray pipes.

The quenching car 4 may contain varying 40 quantities of coke according to the size of the ovens, but will generally vary between twenty and twenty-six thousand pounds, and experience has shown that approximately two-tenths of a gallon of water is all that 45 is necessary to quench one pound of coke under the improved method of this application; when the coke has a temperature of approximately nineteen hundred degrees

Fahrenheit, while at least thirty per cent more water is needed to quench the same 50 quantity of coke under the old method.

By the use of this improved method of quenching the water is permitted to drain away from the coke and the hot steam rising through the tower will produce a stack 55 effect to draw air through the openings 3 and 7 of the tower, as indicated by arrows in the drawings. The air thus drawn into the tower will circulate freely upward through the drained coke to aid in the cooling of the coke.

It will be understood that while I have shown a more or less schematic arrangement of apparatus in the drawings for carrying out my improved method, that such apparatus is only illustrative and that I do not 65 wish to be limited to the use of such apparatus in the use of my method which is expressed in the following claims.

I claim:

1. The method of quenching hot coke which includes intermittently spraying the hot coke with water for relatively short periods, and permitting the coke to drain and cool for relatively long periods between 75 the successive spraying periods.

2. The method of quenching hot coke which includes intermittently spraying the hot coke with water for relatively short periods, and permitting the coke to drain 80 and cool for relatively long periods between the successive spraying periods, and causing an induced flow of air upwardly through the coke during said cooling and draining periods.

3. The method of quenching hot coke which includes the steps of intermittently spraying the hot coke with water and permitting the coke to drain and the residual water on the coke to evaporate between the 90 spraying periods, at least two spraying and two draining periods being used to quench the coke.

In testimony whereof, I have hereunto set my hand.

FRANK F. MARQUARD.